

May 29, 1945.

I. F. BULATKIN

2,376,899

SEALING FACING AND CLOSURE

Filed Aug. 19, 1942

2 Sheets-Sheet 1

Fig. 1a.



Fig. 1.



Fig. 2.



Fig. 4.



Fig. 3.



Fig. 5.



Inventor:

Iliya F. Bulatkin,  
By, Arthur Dwyer, Louisville,  
Attorneys.

May 29, 1945.

I. F. BULATKIN

2,376,899

SEALING FACING AND CLOSURE

Filed Aug. 19, 1942

2 Sheets-Sheet 2



Inventor:

Iliya F. Bulatkin,  
By Cushman, Darby & Cushman

Attorneys.

## UNITED STATES PATENT OFFICE

2,376,899

## SEALING FACING AND CLOSURE

Iliya F. Bulatkin, Baltimore, Md., assignor to  
 Crown Cork & Seal Company, Inc., Baltimore,  
 Md., a corporation of New York

Application August 19, 1942, Serial No. 455,370

6 Claims. (Cl. 215—39)

The present invention relates to an improved sealing facing for container closures, to sealing discs formed from the facing material, and to container closures equipped with the sealing discs.

It is well recognized that material in the nature of plain pulp board cannot be successfully used as a sealing facing for container caps where an effective seal is essential, as, for example, in the bottling of pressure beverages. This is for the reason that due to the irregular surfaces of both the pulp board and the bottle lip, minute openings are bound to exist through which the gases can escape.

In an attempt to increase the efficiency of such sealing media, the pulp board has been provided on its exposed face with a film of wax, with the idea that the wax would conform to the irregularities in the facing material and container lip and thus provide an effective seal. It has been found, however, that such a wax film still affords an unsatisfactory seal. The wax film has to be extremely thin, it has been found, and is inadequate to fill the irregularities against the escape of pressure. It might be thought that by merely using a film of substantial thickness greater sealing efficiency would be afforded, but actually a proper seal is not secured, for the wax either cracks or distorts in the area where it is pressed against the lip of the container, permitting leakage. If the wax is soft, it has a tendency to squeeze out, and if it is hard it has a tendency to fracture by reason of the crowning pressure which usually ranges from 450 to 600 pounds per square inch. Out of a number of containers sealed by means of closures equipped with the pulp board facing with a relatively heavy wax film, a few will hold fairly high pressure without leakage, but most will leak quite readily at low pressures because of the disruption or fracture of the wax. Another very objectionable feature in the use of such heavily waxed discs is that appreciable amounts of wax are left on the container lip.

I have found that the difficulties heretofore attendant on the use of waxed discs can be overcome if fibrous material, preferably in the form of a meshed fibrous fabric, is embedded in the wax film, the fibers serving to sustain the wax against squeezing out and assuring that none will adhere to the container lip when the closure is removed. The object of the present invention is, therefore, to provide an improved and economical sealing facing in the form of cushion material having a coating of wax material on at least one

face thereof, with fibrous material, in the form of ordinary cheesecloth, for example, embedded therein.

The invention will be described with reference to the accompanying drawings, in which:

Figure 1 is a plan view of a fragment of a sheet or strip of facing material in accordance with the invention.

Figure 1a is a section of the facing material of Figure 1 in a partly disassembled relation.

Figure 2 is a plan view of a sealing disc in accordance with the invention.

Figure 3 is a section on line 3—3 of Figure 2.

Figure 4 is a bottom plan view of a cap equipped with the disc of Figures 2 and 3 and with a spot applied to the disc.

Figure 5 is a section on line 5—5 of Figure 4.

Figure 6 illustrates means for applying wax to a web of pulp board and a single web of fibrous material.

Figure 7 shows means for applying wax to a web of pulp board and to webs of fibrous material, one on each face of the pulp board, and

Figure 8 shows means for applying wax to a web of pulp board which has webs of fibrous material preliminarily affixed to both faces thereof.

Referring to Figure 1, reference numeral 10 designates a sheet of cushion material in the nature of pulp board whose thickness is preferably not over .050 inch. Board of less thickness, for example, .030 inch or .040 inch, with proper density, will serve.

Reference numeral 11 designates a coating of wax, which coating has, for example, a thickness on the order of .015 inch. This wax is preferably fairly soft, i. e. plastic, and many suitable species are available, for example, Pale Yellow Amorphoid Paraffin Wax (180° F. melting point) 80, Petrowax (plastic amorphoid paraffin wax from petrolatum) 20, a single wax such as Petrosene A (an amorphoid paraffin of 168° F. melting, refined by Socony Vacuum Oil Co.).

The following formulae may also be mentioned by way of example:

45 *Formula No. 1* Part by weight  
 160° F. M. P. Barnsdall amorphous wax----- 1  
 180° F. M. P. Barnsdall amorphous wax----- 1

50 *Formula No. 2* Parts by weight  
 Piccolite 125 resin ----- 8  
 Butyl stearate (plasticizer) ----- 2  
 160° F. Barnsdall amorphous wax ----- 45  
 55 180° F. Barnsdall amorphous wax ----- 45

## Formula No. 3

|                                       | Parts by weight |
|---------------------------------------|-----------------|
| Butyl stearate (plasticizer)          | 6               |
| Resin piccolite 125                   | 100             |
| 160° F. M. P. Barnsdall amorphous wax | 100             |

## Formula No. 4

|                                                      | Parts by weight |
|------------------------------------------------------|-----------------|
| Opal wax (synthetic wax of Du Pont)                  | 60              |
| Tricresyl-phosphate (plasticizer)                    | 10              |
| Butyl methacrylate (polymer) Du Pont synthetic resin | 30              |
| Talcum (mineral filler)                              | 20              |
| Gilsonite pitch (for color)                          | 2               |

## Formula No. 5

|                                             | Parts by weight |
|---------------------------------------------|-----------------|
| Piccolite 125                               | 40              |
| Butyl methacrylate                          | 12              |
| Abalyn (plasticizer by Hercules Powder Co.) | 20              |
| 180° F. Barnsdall amorphous wax             | 30              |
| Talcum                                      | 30              |

After the wax has been applied to the board and while it is still warm, or after being re-warmed, a web of cheesecloth, as indicated by the reference numeral 12, is applied to the wax with pressure so as to be embedded therein, becoming an integral part of the wax coating as indicated at 13. In Figure 1 it is not intended to imply that the wax 11 and cloth 12 are separate laminae, and it may be assumed that where the cheesecloth appears alone it is just about to be pressed into the wax in the manner suggested in Figure 1a.

Other ways of producing the composite web are shown by way of example in Figures 6 to 8. In Figure 6 reference numeral 20 designates a roll of cheesecloth and 21 a roll of pulp board. The cloth and board are led over heated rolls 22 and 23, respectively, and downwardly through the bite of the same to a winding roll 24. Rolls 22 and 23 are yieldingly urged together and suitably heated and in their bite support a quantity of melted wax 25 in contact with the webs. The webs pick up the wax in suitable thickness and are united thereby, the wax hardening sufficiently before reaching roll 24 so that the windings on the latter will not run together.

In Figure 7 reference numerals 20a and 26 designate rolls of cheesecloth and reference numeral 27 a roll of pulp board. The cheesecloth is led over the heated rolls 22a and 23a and downwardly between the two while the board is led between the cloth webs at the bite of the rolls. Wax is applied as before and the composite web is led to a winding roll as in Figure 6.

In Figure 8 reference numeral 28 designates a composite web comprising a core of pulp board with facings of cheesecloth preliminarily affixed thereto as by paste or glue which may be spot-applied. The web is pulled between the rolls 22b and 23b and the wax bath as by a winding roll disposed below.

It is not necessary that the cheesecloth be completely embedded in the wax so that a smooth wax surface exists and, as a matter of fact, in ordinary practice the fiber strands show and can be felt on the surface, although they are wax-filled.

Cheesecloth has been mentioned as an inexpensive material which is readily applied and which can be obtained in suitable thickness. Its thickness is preferably not more than from about .0050 inch to .0060 inch. Its mesh, which is a secondary factor, may vary, for example, between 32/36 and 24/11 (English system). Ordinary cotton

cheesecloth serves very satisfactorily, but fabrics in the nature of cheesecloth made from any other suitable fibers can be used.

In Figures 1 and 1a only one face of the pulp board body is shown as provided with the reinforced coating. It will be understood, however, that both faces of the board can be identically treated, and ordinarily will be as a matter of convenience in assembling the discs and closures. In Figures 2 and 3 reference numeral 14 designates a sealing disc punched from a sheet or strip coated on both sides, as above described, the two strata of reinforced wax material being indicated at 15 and 16, Figure 3, and the pulp board at 17.

While sealing discs according to the invention may be used with any type of cap, the disc 14 of Figures 2 and 3 is shown in Figures 4 and 5 as assembled in a crown shell 18. If the packaged substance is such that contact with the wax coating would be injurious, a spot may be applied to the exposed face of the disc, such spot being designated by the reference numeral 19, Figures 4 and 5.

When the crown of Figures 4 and 5 is applied to a container, the capping pressure cannot disintegrate and squeeze out the wax coating at the lip, since the fibers hold the wax in place. Microscopic examination of a removed closure shows many hair-like fibers shooting off from the main fibers and assisting the latter to sustain the wax film. The sealing efficiency is usually dependent upon the nature of the paper material and the kind of wax used. If the wax is plastic the sealing efficiency is greater than in the case of hard wax. With a suitable wax, fiber-reinforced, pressures of 100 pounds and over are effectively held.

The pulp board or like material may be wax impregnated prior to coating, or not. A single wax may be used, or a mixture of waxes, or a compound of waxes, or a compound of wax and other modifying materials, such as resins, plasticizers, mineral fillers, pitches, and coloring agents may be used. A single wax or any suitable wax composition is contemplated under the term "wax material" as used in the claims which follow. The invention contemplates broadly the use of fibrous material in any form so long as the fibers are arranged to sustain the coating, but from the standpoints of ease of manufacture and efficiency in use, I prefer to use web material in the nature of cheesecloth. In some situations it may be desirable to use more than one layer of the fibrous mesh material, but ordinarily this will not be the case. While I have shown a solid sealing disc it will be understood that the disc could be annular, if desired. Since the invention is thus susceptible of variation by way of specific materials used and the form of the disc, it will be understood that I do not limit myself in these respects except as in the following claims.

I claim:

1. A container closure having therein a sealing disc comprising a pulp board disc having on its exposed face a film of wax material, and a disc of cheesecloth embedded in said film.

2. A crown cap having fixed therein a sealing disc comprising a pulp board disc having a cheesecloth disc adhesively affixed to the exposed face thereof, and an adherent film of a wax material embedding said cheesecloth disc.

3. For use as material for the sealing discs of container closures, a web of pulp board having on at least one of its faces a film of a wax material, and a web of cheesecloth embedded in said film.

4. For use as material for the sealing discs of container closures, a web of pulp board having a web of cheesecloth adhesively affixed to a face thereof, and an adherent film of a wax material embedding said cheesecloth web.

5. A sealing disc for container closures, said disc comprising a pulp board disc having on at least one of its faces a film of a wax material,

and a disc of cheesecloth embedded in said film.

6. A sealing disc for a container closure, said disc comprising a pulp board disc having a cheesecloth disc adhesively affixed to a face thereof, and an adherent film of a wax material embedding said cheesecloth disc.

ILIIYA F. BULATKIN.